

## UNITED STATES PATENT OFFICE

2,238,553

## DIESEL ENGINE FUEL

Marvin L. Chappell, Berkeley, Calif., assignor to  
 Standard Oil Company of California, San Francisco, Calif., a corporation of Delaware

No Drawing. Application March 14, 1938,  
 Serial No. 195,823

5 Claims. (Cl. 44—9)

This invention relates to fuel boiling above the gasoline range and to primers produced therein for the purpose of lowering its spontaneous ignition temperature when used in internal combustion engines with fuel injection at the end of the compression stroke.

Fuel oil containing such accelerators or primers is used chiefly to operate internal combustion engines of the Diesel or semi-Diesel type in which ignition of the fuel is effected by the heat developed in the compression of the air.

It has been previously proposed to add to Diesel fuel a small percentage of an ignition accelerator of the explosive type, such as peroxides, nitro-compounds, perborates, persulfates and the like, which lower the spontaneous ignition temperatures of the fuel oil itself. However, agents of the explosive type are dangerous to handle, unstable, and may be decomposed after addition to the fuel when stored for a period of time before use.

Now, I have discovered improvements in the product and process for lowering the ignition temperature of Diesel engine fuels, by producing therein diazonium salt reaction products with constituents of the fuel, among which products may be included some compounds probably in the nature of azo compounds, which is accomplished by treating the fuel with a diazonium acid salt at temperatures preferably below 40° F., then neutralizing the treated fuel mixture with a water solution of an alkali hydroxide and finally separating the water containing dissolved salts of reaction from the treated fuel containing the diazonium salt reaction products in solution.

I have discovered that this type of diazonium salt reaction products produced in the fuel by the aforesaid method is stable and sufficiently sensitive to facilitate combustion to the desired degree, the percentage required depending upon the character of the hydrocarbon composition of the fuel and the type of Diesel engine in which the fuel is to be used. For high type compression engines a less percentage of the diazonium salt reaction product is required than with semi-Diesel engines which operate at lower compressions, the quantity required ranging from about .1% to as high as 10% by weight of amine used to make the diazonium acid salt for the treating operation. For Diesel fuels consisting principally of aliphatic hydrocarbons, a smaller amount of diazonium acid salt would be required for the treating operation than when the fuel is composed primarily of carbocyclic hydrocarbons to obtain given cetane numbers.

An object of the invention is to produce a new motor fuel by an improved process of treating petroleum oil or petroleum oil products, with an agent capable of converting a part thereof into primers or lower ignition products of the type resulting from the diazonium salt reaction with constituents in the petroleum oil or petroleum oil products.

Another object of the invention is to produce a new fuel for Diesel type engines with an ignition temperature sufficiently low to suit the engine in which it is to be used.

Various other objects and advantages of the present invention will be apparent from the following example which illustrates in general the preferred method of preparing the new fuel sensitized to the degree necessary for the type of engine in which it is to be used.

Diesel fuel prepared from petroleum oil, petroleum residuum, petroleum distillate or petroleum residuum mixed with distillate, maintained at a temperature below 40° F., preferably at about 32° F., is commingled with an acid water solution of a diazonium acid salt, and thereafter neutralized with a water solution of an alkali with continuous cooling sufficient to maintain the temperature of the mixture below 40° F. until the azo reaction is complete. Thereafter the treated fuel mixture is raised to a higher temperature and the water containing the dissolved salts of the neutralizing reaction is separated from the treated fuel containing the diazonium salt reaction products in solution.

The diazonium acid salt for the treating operation is made by any of the well known methods of treating primary aromatic amine salts at low temperatures with nitrous acid in the presence of a sufficient quantity of acid to form the salt desired. Preferably, a water solution of sodium, potassium or amyl nitrite followed by an addition of acid to decompose the salt, is used to form the nitrous acid required for the di-azo reaction, although any other nitrous acid salts may be used in conjunction with the required quantity of acid to transform the nitrite used into the acid. The acid used to decompose the nitrite salt and also to form the diazonium salt may be hydrochloric, sulfuric, hydrobromic, acetic and the like.

The preferred method of producing a water solution of a diazonium salt and treating the Diesel fuel by this invention is as follows:

93 parts by weight aniline, 121 parts by weight xylylne, or 143 parts by weight naphthylamine is dissolved in 2300 parts by weight of a water solution of hydrochloric acid containing 88 parts by

weight HCl, and then cooled to 32° F. To the above mixture 73 parts by weight nitrite of soda dissolved in 300 parts of water is added slowly with thorough mixing and continuous cooling so that the temperature will not exceed 35° F. until the diazotizing reaction is complete. This water solution of benzenediazonium chloride is then commingled with 4650 parts by weight Diesel fuel, in case 2% of aniline is required to produce the necessary quantity of diazonium salt reaction product to raise the cetane number of the fuel to the required degree. After mixing the benzenediazonium chloride with the Diesel fuel the diazonium salt reaction is completed by neutralizing the excess acid with a water solution of sodium hydroxide or other neutralizing agent at a maintained temperature not to exceed 40° F. Thereafter the water containing dissolved salts of the reaction is separated from the treated fuel containing the diazonium salt reaction products in solution.

The following illustrates the effect of treating a standard Diesel fuel of gas oil stock derived by distillation of California crude petroleum, with varying percentages of diazonium acid salts in terms of aniline used:

| Composition of fuel | Per cent aniline used | Cetane number before treatment | Cetane number after treatment |
|---------------------|-----------------------|--------------------------------|-------------------------------|
| Gas oil stock.....  | 2                     | 41                             | 47                            |
| Do.....             | 5                     | 41                             | 55                            |
| Do.....             | 10                    | 41                             | 68                            |

The above example illustrates one method of treating Diesel fuel to raise the cetane number in which the per cent of diazonium acid salt used may vary through a wide range and the fuel so treated may be compounded with other fuels to increase the cetane number of the mixture.

While the product herein described illustrates a new motor fuel and a process of manufacture thereof, various modifications and changes may be made without departing from the spirit of the invention, and the invention includes all such modifications and changes as appear within the scope of the appended claims.

I claim:

1. The method of increasing the cetane number of a petroleum Diesel oil fraction boiling in the Diesel oil range and suitable for use as a Diesel fuel but having an undesirably low cetane number, which comprises treating said Diesel oil fraction with a diazonium salt at temperatures below about 40° F., in proportion sufficient to form diazonium salt reaction products in said

Diesel oil fraction and to increase the cetane number, neutralizing the resulting mixture, and separating the water containing the dissolved salts of reaction from the Diesel oil fraction containing the diazonium salt reaction products in solution.

2. The method of increasing the cetane number of a petroleum Diesel oil fraction boiling in the Diesel oil range and suitable for use as a Diesel fuel but having an undesirably low cetane number, which comprises reacting said Diesel oil fraction with a diazonium salt at temperatures below about 40° F., in proportion sufficient to form diazonium salt reaction products with constituents of said Diesel oil fraction and to increase the cetane number, neutralizing the resulting mixture, and separating the water containing the dissolved salts of reaction from the Diesel oil fraction containing the diazonium salt reaction products in solution.

3. In a process of lowering the ignition temperature of a Diesel fuel boiling in the Diesel fuel range, the steps which comprise diazotizing a primary aromatic amine salt in a water solution containing acid, treating said Diesel fuel with the resulting diazotized solution, and neutralizing the treated fuel at temperatures below 40° F.

4. The method of increasing the cetane number of a petroleum Diesel oil fraction boiling in the Diesel oil range and suitable for use as a Diesel fuel but having an undesirably low cetane number, which comprises treating said Diesel oil fraction with benzene diazonium chloride at a temperature below about 40° F. in proportion sufficient to form benzene diazonium chloride reaction products in said Diesel oil fraction and increase the cetane number, neutralizing the resulting mixture, and separating the water containing the dissolved salts of reaction from the Diesel oil fraction containing the benzene diazonium chloride reaction products in solution.

5. The method of increasing the cetane number of a petroleum Diesel oil fraction boiling in the Diesel oil range and suitable for use as a Diesel fuel but having an undesirably low cetane number, which comprises reacting said Diesel oil fraction with benzene diazonium chloride at a temperature below about 40° F. in proportion sufficient to form benzene diazonium chloride reaction products with constituents of said Diesel oil fraction and increase the cetane number, neutralizing the resulting mixture, and separating the water containing the dissolved salts of reaction from the Diesel oil fraction containing the benzene diazonium chloride reaction products in solution.

MARVIN L. CHAPPELL.